

Patented Sept. 7, 1926.

1,599,358

# UNITED STATES PATENT OFFICE.

MAX BERGMANN, EUGEN IMMENDÖRFER, AND ALICE IMMENDÖRFER, NÉE GOODSON,  
OF DRESDEN, GERMANY.

## PROCESS FOR REMOVING THE HAIR FROM GREEN HIDES.

No Drawing. Application filed September 13, 1924, Serial No. 737,607, and in Germany September 19, 1923.

It has become known to use alkali- or earth alkali sulphides for removing the hair from green hides. It is further known to use for the same purpose nitrogen bases like 5 ammonia alone, for instance in closed chambers and in the heat. The first mentioned process more or less affects the hair especially the wool, and the last mentioned processes are cumbersome and require expensive installations. It has further been proposed to use a mixture of sodium sulphide and of sodium sulphhydrate to which such 10 quantities of ammonia carbonate are added, that the sodium sulphhydrate is converted into equal parts of sodium sulphide and of ammonia sulphide. Consequently in this process also considerable quantities of active sulphide of sodium remain present and exert their unfavorable, decomposing action 15 on the hair, at the roots as well as at the parts exposed above the skin.

We now have found that the above stated inconveniences can be avoided by using sulphides of inorganic or organic nitrogen 20 bases which are free from active alkali sulphides, the hair, wool and the like being thus well preserved in the slackening process. Either the already formed sulphides of the nitrogen bases may be employed as starting materials and used as they are, or alkali sulphide may be converted with at least the equimolecular or even greater quantities of suitable salts of inorganic or organic nitrogen bases, and the liquids thus obtained be 25 used for the slackening process, said liquids no more containing any active free alkali sulphide.

Further we have found that an unhauling liquid, combined from solutions of ammonia sulphide and soluble silicates, is specially well suited for this purpose. A liquid of this kind frees the hides and skins from hair within a few hours and does not affect the valuable skin substance nor the hair.

### 45 Examples.

1.—To free fleeces from wool the slackening liquid is prepared as follows:

20 liters of commercial ammonia sulphide, 50 200 liters of aqueous ammonia solution (of 0.910 spec. gravity) and 20 hectoliters of water are mixed together. Into this solution the corresponding quantity of sheepskins or fleeces is immersed, the quantity of

steeping liquid amounting for instance to 55 five times the weight of the hides. The temperature is preferably maintained at 25° C., and after 1 to 2 days the skins will release the hair quite readily. The wool remains 60 in a very good condition.

2.—Instead of the free ammonia the corresponding quantity of pyridin (1/2 of 1 liter of technical pyridin for one liter of ammonia solution) is used, the proceeding being otherwise as indicated in Example 65 No. 1.

3.—Instead of the ammonia, carbamide is used, the process being otherwise as indicated in Example No. 1.

4.—For unhauling a set of fleeces or sheepskins a slackening solution is used which contains for 1 cubic meter of water 50 liters of commercial water glass solution and 20 liters of a solution of technical ammonia sulphide. The composition may vary considerably and be, without prejudice, stronger than indicated.

So much of this unhauling liquid is used that the hides are well covered. After 5 to 6 hours already, the mass having been 80 agitated repeatedly, the hides will let loose the hair readily, this loosening of the hair being further improved within 1 to 2 days. The skin is not affected at all but comes out of the process at a very clear state. The 85 wool is of excellent softness and good touch and proves to contain the elastin yet in unaltered state. It differs not in the least from good fleecing.

The treatment of other kinds of hides may 90 be carried out in a similar manner, with convenient modification of the process. In all these cases the working prescriptions for the unhauling process must be adapted to the special working process of the tannery in 95 question and to the desired quality for the leather to be obtained.

Instead of ammonia sulphide such salt mixtures may be employed which when dissolved will form ammonia sulphide, as for 100 instance mixtures of sodium sulphide and ammonium chloride.

Other substances may eventually be added to the slackening liquid.

Having now particularly described and 105 ascertained the nature of our said invention, we declare that what we claim is:

1. A process for unhauling hides consist-

- ing in immersing the hides in a solution containing sulphides of nitrogen bases and being free of active alkali sulphide.
2. A process for unhairing hides consisting in immersing the hides in a solution containing sulphides of inorganic nitrogen bases and being free of active alkali sulphide.
3. A process for unhairing hides consisting in converting alkali sulphide with at least the equimolecular quantity of salts of nitrogen bases into sulphides of said nitrogen bases, and immersing the hides in the solution thus obtained.
4. A process for unhairing hides consisting in converting alkali sulphide with at least the equimolecular quantity of salts of inorganic nitrogen bases into sulphides of said inorganic nitrogen bases, and immersing the hides in the solution thus obtained.
5. A process for unhairing hides consisting in immersing the hides in a solution con-
- taining sulphides of nitrogen bases and soluble silicates.
6. A process for unhairing hides consisting in immersing the hides in a solution containing sulphides of inorganic nitrogen bases and soluble silicates.
7. A process for unhairing hides consisting in immersing the hides in a solution containing ammonium sulphide and a soluble silicate.
8. A process for unhairing hides consisting in converting alkali sulphide with at least the equimolecular quantity of ammonia salt into ammonium sulphide, adding a soluble silicate thereto, and immersing the hides in the solution thus obtained.
- In testimony whereof we have hereunto set our hands.
- Prof. MAX BERGMANN.  
Dr. EUGEN IMMENDÖRFER.  
Dr. ALICE IMMENDÖRFER, née GOODSON.